

## PREPARATION OF QUICK-BREAKING BITUMINOUS EMULSIONS CHARACTERIZED BY IMPROVED DEMULSIBILITY

Edward W. Mertens and James R. Wright, El Cerrito, Calif., assignors to California Research Corporation, San Francisco, Calif., a corporation of Delaware

No Drawing. Filed Jan. 27, 1959, Ser. No. 789,253

8 Claims. (Cl. 252—311.5)

The present invention concerns a new method of preventing impairment of certain critical properties of quick-breaking oil-in-water type bituminous emulsions prior to their actual use in road work and the like. More particularly, it relates to a method of preparing quick-breaking bituminous emulsions from readily emulsifiable asphalts, in such a way that the demulsibility of the finished emulsion is either enhanced, held constant, or at least maintained within the limits set up in the specifications of the trade.

The term "readily emulsifiable asphalts" as employed herein refers to asphalts with acid numbers equal to at least 2.0 and higher, and particularly to asphalts rich in emulsifying acids (naphthenic and/or asphaltic) and characterized by acid numbers in the range from about 3.0 to about 4.0. These asphalts are available on the market in substantial volumes, and since they readily lend themselves for the emulsification in situ with conventional emulsifying bases, such as NaOH or KOH, they could have been regarded as a very attractive source material for the preparation of quick-breaking asphalt-in-water road emulsions. However, in actual practice it has been noted that the emulsions prepared from these asphalts tend to undergo a rapid reduction in demulsibility. In fact, this reduction is often so severe that the emulsified material does not conform to the specifications of the trade, and, being too stable, becomes useless when actually applied to the aggregate. Furthermore, emulsions prepared from these asphalts display poor adhesion property, while their viscosity often undergoes a substantial drop prior to the actual use.

Substitution of neutral electrolytes for a portion of the alkali metal hydroxide base, for instance, substitution of an alkali metal chloride, chromate or the like, does not remedy the situation: true, adhesion may be improved thereby, particularly when using chromates, but demulsibility and viscosity continue to suffer significant drops, particularly if stored for any appreciable length of time at tank temperatures from about 150 to about 170° F., normally maintained in storing asphalt emulsion. In all cases, the higher the proportion of the neutral electrolyte replacing the emulsifying base, the lower is the emulsion viscosity.

The exact causes of the drop of demulsibility and other undesirable fluctuations of emulsion properties are not completely understood, although it is believed that under the warm alkaline conditions obtainable in a storage tank, additional acids are formed in the emulsified asphalt by the hydrolysis of various materials present therein, such as anhydrides, esters, lactones, etc., which could not be saponified, or did not get saponified readily, by the conventional emulsifying base, such as NaOH, in the original emulsification step. These newly formed acids react with the alkaline base remaining in the emulsified asphalts and thus may occasion the drops in demulsibility and viscosity of the emulsion.

It has now been found that the demulsibility of quick-breaking emulsions prepared from readily emulsifiable

asphalts, particularly from those characterized by acid numbers from about 3.0 to about 4.0, can be effectively and significantly improved so as to prevent adverse fluctuations thereof below the acceptable limits set in the specifications of the trade, such as ASTM Specification for Emulsified Asphalt D977-53, which calls for a minimum demulsibility of 60% for Type RS-1 and RS-2 emulsions. This stabilization of demulsibility is achieved by pretreating the asphalt, at temperatures from about 250 to about 325° F. and prior to the emulsification, with a nitrogen-containing material which reacts at these temperatures with carboxylic acids of the asphalt to form amides, for a sufficiently long period of time to cause the lowering of the acid number of the asphalt to at least 1.8 or lower, but not lower than about 0.8, and preferably to a figure in the range from about 1.5 to about 1.0.

Primary and secondary amines, ammonia and any other nitrogen-containing material reacting with a carboxylic acid to form an amide can be thus employed in accordance with the invention in sufficient amounts to convert a portion of the emulsifying acids in the asphalt to amides, leaving, however, enough unconverted free acids to enable subsequent emulsification of the asphalt in water with the aid of conventional emulsifying bases, such as NaOH or KOH.

The amidation treatment can be carried out in any convenient manner. Generally, the amidizing agent is stirred into the asphalt in the storage tank at a temperature within the range from about 250 to about 325° F. With thorough mixing, the reaction is completed within 30 to 60 minutes, as indicated by the measurement of the acid number which now falls within the range from 1.8 to about 0.8. Thereupon the treated material is either stored, or is immediately emulsified in a known manner (employing conventional emulsifying bases), and then may be stored for several days, usually without displaying any inordinately large reduction of demulsibility and viscosity characteristics. Upon prolonged storage (a week or longer) these properties may decrease somewhat but in most cases will remain within the limits of the specifications of the trade, such as ASTM D977-53.

As mentioned above, the amidizing agent (amines, ammonia, and the like) may be admixed to the asphalt in the storage tank; or it may be introduced into the asphalt as it flows from the reduction column at the refinery to the storage tank; or it may be injected into the asphalt while this latter is passed through a recirculation system provided in the storage tank; or yet it may be added to the asphalt-containing crude oil before reduction of this latter. In all instances, the asphalt so treated, after its emulsification with the aid of conventional emulsifying bases (with and without neutral electrolytes), yields satisfactory, storable quick-breaking emulsions whose demulsibility and other properties conform to the specifications of the trade.

Suitable amidizing agents are: (1) primary and secondary aliphatic amines having as many as 18 alkyl carbon atoms, the low molecular weight ones being preferred because of their solubility in water; (2) alkanolamines, e.g., diethanolamine, and the like; (3) primary and secondary mononuclear aromatic amines, e.g., aniline, N-methyl aniline; (4) polyalkylene polyamines, e.g., tetraethylene pentamine; (5) polyalkanol polyamines, e.g., a material known in the trade under the name of "Polyamine T," manufactured by Union Carbide Corp. as a bottoms product of triethanolamine manufacture; (6) other nitrogen-containing materials which at temperatures from about 250 to about 325° F. react with carboxylic acids of the asphalt to form amides, bringing the acid number of the asphalt to 1.8 and lower, for instance, a di-

isocyanate known in the trade under the name of "Nacconate-300" and manufactured by National Aniline Division of Allied Chemical Corporation.

Quick-breaking emulsions prepared from readily emulsifiable asphalts which underwent the afore-described amidation treatment in order to reduce the acidity of these asphalts to 1.8 and lower, but not lower than about 0.8, and preferably between about 1.5 and 1.0, and thus to stabilize or at least to minimize the drop in demulsibility of the emulsions, may contain conventional additives which in their turn tend to enhance different emulsion properties, without impairing the benefits obtained in accordance with the present invention. Among these additives, there may be mentioned neutral electrolytes, such as chlorides, phosphates, chromates, sulfates, nitrates, and the like; likewise, there may be added adhesion promoters, stabilizers, thickeners, dispersing agents, clay, etc.

The improvement of the emulsion properties brought about by the pretreatment of asphalt in accordance with the invention has been demonstrated and confirmed in a large number of tests. In each test series asphalts with acid numbers of 2.0 and higher were pretreated in accordance with the invention prior to the emulsification which thereafter yielded quick-breaking emulsions of an asphalt content between about 50 and 75%, and preferably from about 55 to about 70% by weight; in other words, it gave emulsions coming within the purview of the ASTM Standard Specification D997-53 for Emulsified Asphalt of Type RS-1 and RS-2.

The results of several representative tests of one of said test series are given in Table I below to illustrate the practice and the various advantages of the invention.

A number of amidizing agents were used in these tests in amounts which ranged from 0.06% upwards by weight, based on the asphalt, and preferably from 0.125 to 0.25% by weight. Expressed in percent by weight of the ultimately formed quick-breaking emulsion, these percentages were 0.025% and upwards, and preferably from 0.20 to 0.40%.

The asphalt selected for the tests illustrated in Table I as being typical of those with acid numbers of 2.0 or high-

er, was a California 200-300 penetration-grade asphalt from San Ardo Field (the acid number of this asphalt lies between 3.0 and 3.8). The amidizing agents were thoroughly mixed with the asphalt for 30 minutes at 250° F., and the resulting mixture was emulsified, either immediately or following storage (as indicated in the table). When ammonia was used to amidize the asphalt, shorter treating periods than 30 minutes were required. The emulsions were prepared using 63% of the pretreated asphalt, distilled water and NaOH (0.07%) as the emulsifying base. Conventional neutral electrolytes, namely sodium chloride and sodium chromate, have been employed to replace a portion of the emulsifying base which was NaOH (0.07% by weight of the final emulsion). 15 When not immediately emulsified, the pretreated asphalt was stored at 250° F.

After emulsification, the emulsions were stored overnight for 18 hours at 120° F., and then their demulsibility and viscosity were determined in accordance with the recommended ASTM practice for testing emulsified asphalt (ASTM Standard Method D244-49). In the following table, viscosity is accordingly given in seconds (Saybolt-Furo) at 122° F., and demulsibility in percent (as determined with a 0.02 N calcium chloride solution).

20 Adhesion was also determined after overnight storage using a sample of 100 g. of dry Massachusetts rhyolite passing all through a  $\frac{3}{8}$ " sieve and retained all on a No. 4 sieve. An 8 g. sample of the emulsion, preheated to 120° F., is added to the stone with stirring to insure a good coating. The vessel containing this mixture is placed in an oven for 24 hours at 200° F. and then stirred again to provide a complete coating of the aggregate. A 50 g. sample of the so cured mixture is dropped into a beaker containing 400 cc. of boiling distilled water for one minute, again with stirring at a rate of 60 r.p.m. The beaker is then withdrawn from the hot plate, any floating asphalt film removed, and the rhyolite sample withdrawn and dried, whereupon the area of the stone still coated with asphalt is estimated (in percent, average).

25 30 35 40 Adhesion is considered to be satisfactory when at least 75% of all aggregate surface remains coated by asphalt.

TABLE I  
Effect of amidation of asphalt on properties of quick-breaking emulsions

| Run No. | Amidizing Agent            |                            | Neutral Electrolyte              |                            | Properties Determined After 18 Hours at 120° F. |                                                      |                     |
|---------|----------------------------|----------------------------|----------------------------------|----------------------------|-------------------------------------------------|------------------------------------------------------|---------------------|
|         | Name                       | Percent by Wt. of Emulsion | Name                             | Percent by Wt. of Emulsion | Viscosity, SSF/122° F.                          | In Percent Demulsibility (0.02 N CaCl <sub>2</sub> ) | Adhesion in Percent |
| 1       |                            |                            |                                  |                            | 155                                             | 48                                                   |                     |
| 2       |                            |                            | Na <sub>2</sub> Cl               | 0.16                       | 337                                             | 75                                                   | 20                  |
| 3       | Diethylene Triamine        | 0.20                       | Na <sub>2</sub> Cl               | 0.16                       | -----                                           | 99                                                   | 70                  |
| 4       |                            |                            | Na <sub>2</sub> CrO <sub>4</sub> | 0.22                       | -----                                           | 70                                                   | 65                  |
| 5       | Tetraethylene Pentamine    | 0.25                       | Na <sub>2</sub> CrO <sub>4</sub> | 0.22                       | 206                                             | 90                                                   | 85                  |
| 6       |                            |                            | Na <sub>2</sub> CrO <sub>4</sub> | 0.20                       | 247                                             | 67                                                   | 65                  |
| 7       | Aniline                    | 0.40                       | Na <sub>2</sub> Cl               | 0.16                       | 397                                             | 87                                                   | 30                  |
| 8       | Armeeen HTD <sup>2</sup>   | 0.25                       | Na <sub>2</sub> CrO <sub>4</sub> | 0.16                       | -----                                           | 97                                                   | 40                  |
| 9       | Polyamine T <sup>3</sup>   | 0.25                       | Na <sub>2</sub> CrO <sub>4</sub> | 0.20                       | 235                                             | 98                                                   | 85                  |
| 10      | do <sup>3</sup>            | 0.10                       | Na <sub>2</sub> CrO <sub>4</sub> | 0.20                       | 441                                             | 94                                                   | 90                  |
| 11      | Polyamine T                | 0.05                       | Na <sub>2</sub> CrO <sub>4</sub> | 0.20                       | 496                                             | 88                                                   | 95                  |
| 12      | do                         | 0.025                      | Na <sub>2</sub> CrO <sub>4</sub> | 0.20                       | 433                                             | 71                                                   | 75                  |
| 13      | do                         | 0.50                       | Na <sub>2</sub> CrO <sub>4</sub> | 0.20                       | (?)                                             | (?)                                                  | (?)                 |
| 14      | do                         | 1.00                       | Na <sub>2</sub> CrO <sub>4</sub> | 0.20                       | (?)                                             | (?)                                                  | (?)                 |
| 15      |                            |                            | Na <sub>2</sub> CrO <sub>4</sub> | 0.20                       | 107                                             | 61                                                   | 75                  |
| 16      | Nacconate 300 <sup>4</sup> | 0.05                       | Na <sub>2</sub> CrO <sub>4</sub> | 0.20                       | 368                                             | 71                                                   | 70                  |
| 17      | do <sup>4</sup>            | 0.25                       | Na <sub>2</sub> CrO <sub>4</sub> | 0.20                       | 95                                              | 97                                                   | -----               |
| 18      | Ammonia                    | (5)                        | Na <sub>2</sub> CrO <sub>4</sub> | 0.20                       | 157                                             | 68                                                   | -----               |
| 19      | do                         | (6)                        | Na <sub>2</sub> CrO <sub>4</sub> | 0.20                       | 202                                             | 66                                                   | 75                  |
| 20      | Diethylene Triamine        | 0.05                       | Na <sub>2</sub> CrO <sub>4</sub> | 0.20                       | 428                                             | 74                                                   | 70                  |

<sup>1</sup> Following the amidation treatment, asphalt was stored 64 hours at 250° F.

<sup>2</sup> High molecular weight fatty amine material derived from hydrogenated tallow, manufactured and sold by Armour & Co.

<sup>3</sup> Bottoms product from the manufacture of triethanolamine, sold by Union Carbide Corporation.

<sup>4</sup> Diphenyl methane-4,4'-diisocyanate, manufactured and sold by National Aniline Division of Allied Chemical Corporation.

<sup>5</sup> Ammonia treatment lasted 5 and 15 minutes, respectively.

<sup>6</sup> Expressed as 100% active material.

<sup>7</sup> Emulsion broke during the 18 hours of storage.

The results presented in Table I definitely bring out the benefits of the amidation pretreatment of asphalts which have acid numbers of more than about 2.0, carried out in accordance with the present invention. When the asphalt was emulsified using sodium hydroxide alone (run No. 1), the demulsibility determined after overnight storage of 18 hours at 120° F. was quite low (48%) and failed to conform with the specifications of the trade for quick-breaking emulsions (ASTM D977-53). The use of neutral electrolytes, chlorides and chromates, as replacements for a portion of sodium hydroxide while

been used as neutral electrolytes, replacing a portion of the sodium hydroxide emulsifying base. Emulsification was carried out with distilled water as the external phase. After the emulsification, the emulsions were left to stand and their properties (viscosity, demulsibility and adhesion) determined upon 18 hours of overnight storage. Following additional storage which lasted from 8 to 12 days, demulsibility and viscosity determinations were repeated. All of these determinations were carried out in the same manner as described in connection with the data in Table I.

TABLE II  
*Effect of conditions of amidation on demulsibility and storage stability of emulsions*

| Run No. | Percent by Wt. of Amidizing Agent <sup>1</sup> | Neutral Electrolytes             |                             | Conditions of Amidation |                 | After 18 Hours at 120° F. |                        |                   | On Further Storage at 120° F. |           |               |
|---------|------------------------------------------------|----------------------------------|-----------------------------|-------------------------|-----------------|---------------------------|------------------------|-------------------|-------------------------------|-----------|---------------|
|         |                                                | Kind                             | Percent by Wt. <sup>2</sup> | Temp., °F.              | Time in Minutes | Viscosity, SSF/122° F.    | Demulsibility, Percent | Adhesion, Percent | Days                          | Viscosity | Demulsibility |
| 1       | 0.20                                           | NaCl                             | 0.16                        | 220                     | 15              | (6)                       | (6)                    | (6)               | (6)                           | (6)       | (6)           |
| 2       | 0.20                                           | NaCl                             | 0.16                        | 220                     | 10              | 19                        | 97                     | 70                | 7                             | (7)       | (7)           |
| 3       | 0.20                                           | NaCl                             | 0.16                        | 220                     | 5               | 24                        | 98                     | 60                | 7                             | (7)       | (7)           |
| 4       | 0.10                                           | NaCl                             | 0.16                        | 220                     | 15              | 58                        | 96                     | 70                | 7                             | (7)       | (7)           |
| 5       | 0.15                                           | NaCl                             | 0.16                        | 220                     | 15              | 25                        | 98                     | 50                | 7                             | (7)       | (7)           |
| 6       | 0.25                                           | NaCl                             | 0.16                        | 220                     | 15              | 24                        | 99                     | 50                | 7                             | (7)       | (7)           |
| 7       | 0.30                                           | NaCl                             | 0.16                        | 220                     | 10              | (6)                       | (6)                    | (6)               | 7                             | (6)       | (6)           |
| 8       |                                                | NaCl                             | 0.16                        |                         |                 | 255                       | 78                     | 45                | 12                            | 284       | 65            |
| 9       | 0.10                                           | Na <sub>2</sub> CrO <sub>4</sub> | 0.16                        | 250                     | 30              | 172                       | 99                     | 75                | 12                            | 160       | 90            |
| 10      | 0.05                                           | Na <sub>2</sub> CrO <sub>4</sub> | 0.16                        | 250                     | 30              | 381                       | 90                     | 65                | 12                            | 486       | 93            |
| 11      | 0.025                                          | Na <sub>2</sub> CrO <sub>4</sub> | 0.16                        | 250                     | 30              | 365                       | 90                     | 70                | 7                             |           | 85            |
| 12      | 0.20                                           | Na <sub>2</sub> CrO <sub>4</sub> | 0.22                        | 220                     | 10              | 14                        | 98                     | 35                | 7                             | (7)       | (7)           |
| 13      | 0.25                                           | NaCl                             | 0.22                        | 250                     | 30              | 206                       | 90                     | 85                | 7                             | 307       | 97            |
| 14      |                                                | NaCl                             | 0.22                        |                         |                 |                           | 70                     | 65                | 10                            |           | 66            |

<sup>1</sup> Expressed as 100% active material in percent by weight of the finished emulsion.

<sup>2</sup> Expressed as percent by weight of the finished emulsion.

<sup>3</sup> Following the amidation treatment, the asphalt stored for 7 days at 250° F.

<sup>4</sup> Following the amidation treatment, the asphalt stored for 4 days at 250° F.

<sup>5</sup> Following the amidation treatment, the asphalt stored for 2 days at 250° F.

<sup>6</sup> Emulsion broke on overnight storage.

<sup>7</sup> Emulsion broken.

providing the same concentration of sodium ions, although it raised demulsibility somewhat (runs 2, 4, 6 and 15), could never raise it above about 75% (run No. 2). Furthermore, the application of chlorides, as contrasted with chromates, not only had little effect on, but, in fact, appeared to depress the adhesion property (run No. 2).

Contrasted with these unsatisfactory data, the amidation treatment significantly improved the demulsibility, raising it as much as 100% (e.g., runs 8, 9, 10 and 17), and in all instances by not less than 25%, provided the amidizing agent was being employed in a sufficient concentration to bring the acid number down to 1.8 and lower, but, in all events, not lower than about 0.8, and preferably between about 1.5 and 1.0. When an insufficient quantity of the amidizing agent was employed (as in runs 12, 16, 18 and 19), so that the acid number of the asphalt remained above 2.0, demulsibility barely conformed with the specifications and tended to drop down upon extended storage beyond the specified minimum of 60%. When asphalt treated in accordance with the invention was stored, the demulsibility of the emulsions eventually prepared therefrom rose apparently due to the completeness of the amidation treatment. However, when too high a concentration of the amidizing agent was employed (e.g., in runs 13 and 14), storage stability was adversely affected and the emulsion collapsed.

The effect of the conditions of amidation, namely, the temperature and the duration of amidation treatment, on the stability of the final asphalt emulsion is made apparent by the data shown in next Table II.

The emulsions which provided the data for this table have been prepared from the same San Ardo type asphalt pretreated at 220° F. for 5, 10 and 15 minutes with diethylenetriamine selected as an exemplary amidizing agent. Sodium chloride and sodium chromate have again

The data in Table II clearly show that at temperatures outside the operative range from about 250 to about 325° F. the emulsions lack storage stability and break down, either overnight or in less than one week (runs 1, 2, 3, 4, 5, 6, 7 and 12). On the contrary, when the asphalt is amidized within the operative range of temperatures, its emulsions display satisfactory demulsibility and viscosity, and, consequently, an adequate stability in storage. The test results also show that the longer the asphalt is stored following the amidation treatment, the higher is the demulsibility of the emulsions prepared therefrom.

The beneficial effects of the amidation treatment on the demulsibility and viscosity of quick-breaking emulsions prepared from asphalts characterized by acid numerals equal to at least 2.0, and the reduced tendency of these two properties to deteriorate upon storage are additionally illustrated by the data in Table III, obtained in a series of test runs for which the same San Ardo type asphalt was employed. This asphalt was pretreated, using the previously mentioned amidizing material "Polyamine T" purchased from Union Carbide Corp. for 30 minutes at 250° F., whereupon the treated asphalt was stored for 64 hours at 250° F. After this, emulsions were prepared in accordance with the formula: 63% of treated asphalt, 0.07% sodium hydroxide, 0.20% sodium chromate, and distilled water to make up 100% by weight. The resulting emulsions were stored overnight (18 hours) at 160° F., and then their properties, namely, viscosity, demulsibility and adhesion, were determined, using the same methods as described in connection with the data of Tables I and II. Viscosity and demulsibility determinations were repeated after further storage of the emulsions at 160° F. for different periods of time. The results of these determinations are all tabulated in the following Table III and point

out that the amidation treatment in accordance with the invention prevents a runaway deterioration of these important emulsion characteristics.

8  
an acid number of at least 2.0, which comprises intimately contacting said asphalt at a temperature from about 250 to about 325° F. with a nitrogen-containing material

TABLE III  
Effect of prolonged storage on emulsion properties

| Run No. | Polyamine T in Percent by Wt. <sup>1</sup> | Properties after Storage for 18 Hours at 160° F. |                                                      |                     | Properties after Extended Storage at 160° F. |     |     |     |     |                     |     |     |     |    |
|---------|--------------------------------------------|--------------------------------------------------|------------------------------------------------------|---------------------|----------------------------------------------|-----|-----|-----|-----|---------------------|-----|-----|-----|----|
|         |                                            | Viscosity in SSF/122° F.                         | Demulsibility in Percent (0.02 N CaCl <sub>2</sub> ) | Adhesion in Percent | Viscosity, Days                              |     |     |     |     | Demulsibility, Days |     |     |     |    |
|         |                                            |                                                  |                                                      |                     | 2                                            | 3   | 6   | 8   | 13  | 2                   | 3   | 6   | 8   | 13 |
| 1       |                                            | 231                                              | 57                                                   | 65                  | 202                                          | 204 | 231 | 225 | 230 | 49                  | 52  | 44  | 39  | 34 |
| 2       | 0.08                                       | 342                                              | 93                                                   | 75                  | 333                                          | 366 | 375 | 402 | 398 | 69                  | 70  | 67  | 53  | 53 |
| 3       | 0.10                                       | 367                                              | 91                                                   | 80                  | 351                                          | 415 | 409 | 433 | 409 | 84                  | 75  | 70  | 64  | 48 |
| 4       | 0.12                                       | 398                                              | 94                                                   | 85                  | 360                                          | 439 | 469 | 447 | 88  | 89                  | 84  | 74  | 62  |    |
| 5       | 0.14                                       | 494                                              | 96                                                   | 90                  | 499                                          | 625 | 549 | 566 | 565 | 94                  | 84  | 84  | 74  | 62 |
| 6       | 0.16                                       | 497                                              | 97                                                   | 95                  | 540                                          | 503 | 518 | 595 | 515 | 88                  | 95  | 76  | 69  | 52 |
| 7       | 0.18                                       | 502                                              | 97                                                   | 95                  | 488                                          | 510 | 524 | 97  | 94  | 95                  | 80  | 80  | 56  |    |
| 8       | 0.20                                       | 350                                              | 99+                                                  | 95                  | 336                                          | 418 | 464 | 516 | 99+ | 99                  | 98  | 96  | 72  |    |
| 9       | 0.22                                       | 85                                               | 99+                                                  | 95                  | 95                                           | 156 | 236 | 319 | 98  | 99+                 | 98  | 97  | 91  |    |
| 10      | 0.25                                       | 124                                              | 99+                                                  | 95                  | 130                                          | 204 | 315 | 385 | 99  | 99                  | 94  | 94  | 90  |    |
| 11      | 0.30                                       | 30                                               | 99+                                                  | 90                  | 28                                           | (?) | (?) | (?) | (?) | 98                  | (?) | (?) | (?) |    |

<sup>2</sup> Emulsion broken.

As contrasted with the rapidly decreasing demulsibility of an emulsion prepared without pretreating the asphalt with Polyamine T (run No. 1), demulsibility of emulsion from the treated asphalt continues to conform with the specifications of the trade (is higher than 60%) after 8 days of storage, provided the amidizing agent has been employed in an amount sufficient to lower the acid number of asphalt to 1.8 and lower, but not lower than about 0.8. Viscosity likewise remains high after 1 to 2 weeks of storage, and if too high (higher than 400 SSF/122° F.), may be reduced to the specified limits by conventional methods.

The results of Table III unambiguously indicate that demulsibility is enhanced and does not drop significantly after a whole week of storage at temperatures in the range of from 150 to 170° F. conventionally employed by the trade in storing emulsified asphalt. Furthermore, even upon longer storage, demulsibility in many an instance remains within the minimum prescribed in the specifications.

The aforesaid description of the invention clearly indicates the several advantages in using the amidizing treatment for asphalts with acid numbers of 2.0 and higher. This treatment permits production of quick-breaking emulsions of improved demulsibility, viscosity and adhesion, capable of being stored without significant impairment of these properties, which could not be done in the past. By thus remaining within the limits set forth for these properties in the existing specifications for quick-breaking paving and like emulsions, these materials are made acceptable to the trade.

Provided that the amidation treatment is applied at temperatures from about 250 to about 325° F., and for a period of time from 30 to 60 minutes, it may be immediately followed by the preparation of the emulsion in conventional fashion, and thus becomes a part of a continuous process which does not involve an unnecessary loss of time or require special "aging" in storage before the emulsification to insure that sufficient amidation and, consequently, sufficient reduction of the acid number occurred.

Of course, it is to be understood that the invention as set forth in the aforesaid description is not to be limited to any specific amidation agent, or any particular neutral electrolyte, whether employed in the examples or mentioned elsewhere in the description hereinabove. The examples merely serving to illustrate the operativeness. Thus, the invention is limited only by the definitions of the following claims.

What is claimed is:

1. A method of treating an asphalt characterized by

capable to form amides with the carboxylic acids present in the asphalt at these temperatures, said nitrogen-containing material being contacted with the asphalt in an amount and for a period of time sufficient to reduce the acid number of said asphalt to a figure within the range from 1.8 to not lower than about 0.8.

2. A method of treating an asphalt characterized by an acid number of at least 2.0, which comprises intimately contacting said asphalt at a temperature from about 250 to about 325° F. with a nitrogen-containing material capable to form amides with the carboxylic acids present in the asphalt at these temperatures, said nitrogen-containing material being contacted with the asphalt in an amount and for a period of time sufficient to reduce the acid number of said asphalt to a figure within the range from about 1.5 to about 1.0.

3. A method as defined in claim 1, wherein the reaction between the nitrogen-containing material and the carboxylic acids present in the asphalt is carried out at a temperature from about 250° F. to about 325° F. for at least 30 minutes.

4. A method of treating an asphalt characterized by an acid number of at least 2.0, which comprises intimately contacting said asphalt at a temperature from about 250 to about 325° F. with an amino-nitrogen-containing material capable to form amides with the carboxylic acids present in the asphalt at these temperatures, said amino-nitrogen-containing material being contacted with the asphalt in an amount and for a period of time sufficient to reduce the acid number of said asphalt to a figure within the range from 1.8 to not lower than 0.8.

5. A method of treating an asphalt characterized by an acid number of at least 2.0, which comprises intimately contacting said asphalt at a temperature from about 250 to about 325° F. with an amino-nitrogen-containing material capable to form amides with the carboxylic acids present in the asphalt at these temperatures, said amino-nitrogen-containing material being contacted with the asphalt in an amount and for a period of time sufficient to reduce the acid number of said asphalt to a figure within the range from about 1.5 to about 1.0.

6. A method as defined in claim 4, wherein the reaction between the amino-nitrogen-containing material and the carboxylic acids present in the asphalt is carried out at a temperature from about 250° F. to 325° F. for at least 30 minutes.

7. A process for the production of quick-breaking asphalt emulsions, which comprises intimately contacting at a temperature from about 250° to 325° F. for at least

30 minutes an asphalt characterized by an acid number of at least 2.0 with an amino-nitrogen-containing material which reacts at these temperatures with the carboxylic acids in said asphalt to form amides, said material being added to the asphalt in a sufficient amount to reduce the acid number thereof to a figure in the range from 1.8 to not lower than about 0.8, and emulsifying from about 50 to about 75% by weight of the resultant product mixture in water with an alkali metal-emulsifying base to produce an asphalt-in-water emulsion characterized by viscosity which conforms with ASTM Specification D-977-53 for rapid-setting emulsified asphalt, and has a minimum demulsibility of 60%.

8. A process for the production of quick-breaking asphalt emulsions, which comprises intimately contacting at a temperature from about 250° to 325° F. for at least 30 minutes an asphalt characterized by an acid number of at least 2.0 with an amino-nitrogen-containing material which reacts at these temperatures with the car-

15

boxylic acids in said asphalt to form amides, said material being added to the asphalt in a sufficient amount to reduce the acid number thereof to a figure in the range from 1.8 to not lower than about 0.8, and emulsifying from about 50 to about 75% by weight of the resultant product mixture in water with an alkali metal-emulsifying base to produce an asphalt-in-water emulsion which, after having been stored for one week at 160° F., conforms with respect to its viscosity to ASTM Specification D-977-53 for rapid-setting emulsified asphalt, and has a minimum demulsibility of 60%.

## References Cited in the file of this patent

## UNITED STATES PATENTS

|           |                |                |
|-----------|----------------|----------------|
| 2,317,959 | Johnson et al. | Apr. 27, 1943  |
| 2,585,336 | McCoy          | Feb. 12, 1952  |
| 2,652,341 | Craig          | Sept. 15, 1953 |
| 2,819,228 | Dell           | Jan. 7, 1958   |